

## UNITED STATES PATENT OFFICE.

SHINJIRO HORII, OF TOKYO, JAPAN.

## STENCIL SHEET.

No Drawing.

Application filed May 18, 1926. Serial No. 109,974.

This invention relates to improvements in stencil sheets of the type commonly used for autographic and typewriting duplication, consisting of a sheet of fibrous material 5 coated or impregnated with a coating composition including esters of polysaccharides and chlorinated naphthalene.

The object of the present invention is to provide an improved stencil sheet, adapted 10 for stencilization by pressure, which offers a considerably great resistance to the atmospheric influence on using or storing and gives a large number of clear and sharp copies.

In carrying out the invention, a base of 15 open porous material, such as yoshino paper, is coated or impregnated with a coating composition including esters of polysaccharides, such as mannan acetate, cellulose acetate and cellulose nitrate, and chlorinated naphthalene in solution together with or without a 20 tempering agent such as oils, fats, fatty acids and waxes. The coating operation is carried out in the usual manner.

The proportions of the ingredients of the 25 composition may vary according to several circumstances, an example being as follows:—

|                                | Parts by weight. |
|--------------------------------|------------------|
| Cellulose nitrate, 5% solution | 100              |
| Chlorinated naphthalene        | 20               |
| Stearine                       | 5                |
| Castor oil                     | 5                |

To this may be added, if desired, a sufficient quantity of a suitable coloring matter. 35 The term "esters of polysaccharides" is intended to include not only one of definite

esters of polysaccharides, but also a mixture of them.

According to the present invention, on using the coating composition not hitherto 40 employed for the same purpose, the coated sheet is practically permanent for an extended period of time and produces thereon a clear writing by the pressure of a hand stylus or the blow of a writing machine, giving 45 a large number of copies when the sheet is used in the ordinary manner, i. e. in a stencil-duplicating machine.

What I claim is:—

1. As a new article of manufacture, a stencil sheet made of a base of fibrous material, and an impregnating composition comprising esters of polysaccharides and chlorinated naphthalene. 50

2. As a new article of manufacture, a stencil sheet made of a base of fibrous material, and an impregnating composition comprising esters of polysaccharides, chlorinated naphthalene and a tempering agent. 55

3. As a new article of manufacture, a stencil sheet made of a base of fibrous material, and an impregnating composition comprising the following ingredients: 60

|                                | Parts by weight. |
|--------------------------------|------------------|
| Cellulose nitrate, 5% solution | 100              |
| Chlorinated naphthalene        | 20               |
| Mannan acetate, 10% solution   | 20               |
| Stearine                       | 5                |
| Castor oil                     | 5                |

In testimony whereof I affix my signature.

SHINJIRO HORII.